# EUROPEAN PATENT SPECIFICATION

(11) **EP 0 036 252 B1**
(45) Date of publication and mention of the grant of the patent: **16.01.1985**
(21) Application number: 81300721.8
(22) Date of filing: 20.02.1981
(51) Int. Cl.: D06P 5/12, D06P 5/15, D06P 3/54

(54) **Textile printing process**
Verfahren zum Bedrucken von Textilien
Procédé d'impression de textiles

(30) Priority: 13.03.1980 GB 8008597; 29.04.1980 GB 8014139
(43) Date of publication of application: 23.09.1981
(73) Proprietor: IMPERIAL CHEMICAL INDUSTRIES PLC, London SW1P 3JF (GB)
(72) Inventor: Provost, John Reginald, Ecclestone, nr. Chorley, Lancashire (GB)
(74) Representative: Beton, John Lonsdale

## Description

This invention relates to an improved process for the resist or discharge printing of synthetic textile materials.

Resist printing is a method of textile printing in which an undyed textile material is first printed with a substance (the resist) which prevents the uptake or fixation of a subsequently applied dyestuff, so that there is obtained a white pattern on a coloured ground, or a pattern of contrasting colour to the ground by incorporating suitable dyestuffs or colour-producing substances in the resist print paste.

Discharge printing is a method of textile printing in which dyed textile material is printed with a chemical composition (the discharge) that destroys the dyestuff locally to give a white pattern, or in which a second dyestuff, applied simultaneously with the discharge, produces a pattern of contrasting colour.

GB-A-1543724 describes and claims a process for producing discharge printing effects in a coloured ground shade on a synthetic textile material, which comprises applying to that area of the material where the ground shade and the discharge effect are wanted one or more disperse dyes which contain at least one carboxylic ester group but are free from carboxylic acid and sulphonic acid groups, and in a separate stage applying to the material where the discharge effect is wanted a printing paste which is alkaline or becomes alkaline on heating or steaming and which does not contain any reducing agent, thereafter heating or steaming the material and thereafter washing the material.

The above process is typically carried out in the following 7 stages in which the textile material is:-
1. Printed with an alkaline print paste.
2. Dried.
3. Padded with the disperse dyestuff.
4. Dried.
5. Heat treated or steamed.
6. Washed.
7. Dried.

Alternatively, stages 1 and 3 can be reversed, so that the dyestuff is applied to the textile material before the alkaline print paste.

During stage 5, in which the textile material is subjected to the action of heat or steam, the disperse dyestuff in contact with the alkali is converted into a water-soluble form, whilst the disperse dyestuff which is not in contact with the alkali is fixed on the textile material. The water-soluble form of the dyestuff is then removed from the textile material by the washing treatment of stage 6.

It would be desirable if, in the above process, the first drying operation (stage 2) could be eliminated so that stage 1 is followed immediately by stage 3. This "wet-on-wet" process would have the advantages that the process has one stage less, with consequent saving in drying plant occupation time, and also the saving in the energy used to effect drying.

However, using printing pastes containing the alkaline agents which are normally employed, i.e. sodium hydroxide, sodium carbonate, sodium bicarbonate or potassium carbonate, it is found that the "wet-on-wet" technique gives prints having poor definition, because the alkali bleeds out of the print paste during the subsequent drying and fixation stages to give an unsightly dull white halo at the boundary between the originally applied alkaline resist and the subsequently applied dyestuff. This effect is known as "haloing", and prints which exhibit it are not commercially acceptable.

GB-A-1481741 describes the production of multicolour effects using alkali sensitive disperse dyes of a different type to GB-A-1543724 applied in conjunction with alkaline agents.

It has now been found that wet-on-wet resist or discharge prints having sharp definition between the different coloured areas of the print can be obtained if the alkali used in the print paste is sodium or potassium silicate and if specific types of alkali dischargeable dyestuffs are applied.

According to the present invention there is provided a process for producing resist or discharge printing effects on a synthetic textile material which comprises applying to the textile material, in either order (i) an alkaline printing paste which may contain one or more disperse dyestuffs free from sulphonic acid, carboxylic acid and carboxylic acid ester groups, the said dyestuffs being unaffected by alkali at the concentration present, and (ii) a printing paste or passing liquor containing at least one alkali dischargeable disperse dyestuff free from sulphonic acid and carboxylic acid groups, and free from carboxylic acid ester groups which if hydrolysed would leave free carboxylic acid groups attached to the dyestuff molecule, thereafter heating or steaming the material and thereafter washing the material characterised by the presence of sodium or potassium silicate in (i), a carboxylic acid in (ii), and without drying between the application of (i) and (ii).

The alkali-dischargeable dyestuffs which are used in the process according to the present invention may be broadly classified as follows:
A. Dyestuffs which contain one or more lactone rings which open in the presence of alkali with formation of the water-soluble alkali metal salts of the corresponding hydroxy carboxylic acid. Opening of the lactone ring may be accompanied by destruction of the chromophoric system of the dyestuff.
   Examples of this class are the dyestuff of the formula: Yellow which is disclosed in DE-A-2440405, and the dyestuff of formula: Orange which is disclosed in GB-A-1568231.
   Also in this general class are the dyestuffs of the formulae: Bluish-red Bluish-red Bluish-red Bluish-red Bluish-red
   These unsymmetrically substituted compounds having the above-disclosed formulae may be obtained by reaction of equimolar quantities of hydroquinone and a compound of formula: wherein A is hydroxyl, O-acyl or halogen; B is hydrogen, lower alkyl or aryl and R is phenyl which may carry one or more substituents, for example, lower alkyl, lower alkoxy, hydroxy, chloride or bromine. In this specification the term "lower alkyl" and "lower alkoxy" mean alkyl and alkoxy groups respectively which contain 1 to 4 carbon atoms. The reaction may be carried out either in the absence of a solvent or in the presence of a high boiling solvent such as di- or tri-chlorobenzene to give the intermediate of formula: which is subsequently reacted with a compound of formula: wherein A and B have the previously defined meanings and R¹ is phenyl which may carry one or more substituents, R¹ being different to R, to give a compound of formula: which is then oxidised, preferably in situ by using nitrobenzene as reaction solvent or by treatment with an oxidising agent such as hydrogen peroxide in acetic acid, to give the desired dyestuff of formula:
   There may also be used in the process of the present invention the dyestuff of formula: Orange which is disclosed in EP-A-23080.
   Other dyestuffs in class A which may be used in the present process are those which contain the coumarin ring system.
B. Methine dyestuffs containing at least one group, for example the dyestuff of formula: Yellow which is disclosed in FR-A-1551030, and the dyestuff of formula: Yellow which is disclosed in US-A-2850520.
C. Azo dyestuffs derived from anilines having at least two electron-withdrawing groups ortho and/or para to the amino group as diazo components and para-coupling amine coupling components, for example Violet Bluish-red X = H or OCH₃ Navy blue the first two of which are disclosed in GB-A-852493, and the last in GB-A-1050675.
D. Dyestuffs containing groups which are capable of water-soluble salt formation in the presence of strong alkali, including azopyridone dyestuffs and dyestuffs containing phenolic hydroxyl groups or primary or secondary sulphonamide groups, for example: both of which are disclosed in GB-A-1256093;
   the dyestuff of formula: Orange which is disclosed in GB-A-1398741
   the dyestuff of formula: Yellow which is C.I. Disperse Yellow 42;
   the dyestuff of formula: Yellow which is disclosed in GB-A-1016246;
   the anthraquinone dyestuff of formula: Orange which is disclosed in FR-A-1371626, and the pyridone dyestuffs of formulae: Yellow Yellow both of which are disclosed in GB-A-1095829.
E. Dyestuffs derived from 2-aminothiophenes as diazo components and para-coupling amines as coupling components, the thiophene nucleus being substituted by at least two electron-withdrawing groups, for example: Blue Bluish-green these dyestuffs being disclosed in GB-A-1394367 and 1394368, respectively.
F. Azo dyestuffs derived from 2-amino-5-nitrothiazole as diazo component and a para-coupling amine as coupling component, for example the dyestuffs of formulae: Navy-blue Blue Blue which are all disclosed in GB-A-723933;
   the dyestuff offormula: Blue which is disclosed in US-A-2790791, and the dyestuff of formula: Blue which is disclosed in GB-A-840903.

Also usable in the process and having excellent alkaline discharge properties are the miscellaneous dyestuffs C.I. Disperse Violet 88, C.I. Disperse Yellow 180, C.I. Disperse Violet 48, C.I. Disperse Blue 92, C.I. Disperse Yellow 93, C.I. Disperse Yellow 201, C.I. Disperse Yellow 88, C.I. Disperse Yellow 210, C.I. Disperse Red 203 and C.I. Disperse Yellow 202.

Other dyestuffs which may be used in the present process are those which discharge only partially (i.e. do not give a white discharge) and which do not leave a weak enough stain to allow all shades of illumination to be used, but which do show an even residual shade that allows the use of such dyestuffs for limited illuminated shades and which may be used for shading purposes.

Examples of such dyestuffs are (with reference to the previously defined classes):
In Class A: Bluish-red which may be prepared as described previously for similar dyestuffs in Class A.
In Class C:
   The dyestuff of formula: Blue which is disclosed in GB-A-1080480.
   The dyestuff of formula: Greenish-navy which is disclosed in GB-A-952468.
   The dyestuff of formula: Red which is disclosed in GB-A-1225221.
   The dyestuff of formula: Red . which is disclosed in FR-A-1264090;
   and the dyestuff of formula: Reddish-blue which is disclosed in GB-A-1140214.
In Class D:
   The dyestuff of formula: Yellow which is disclosed in GB-A-825377;
   the dyestuff of formula: Scarlet which is disclosed in GB-A-862269;
   the dyestuff of formula: Golden yellow which is disclosed in GB-A-1020303;
   the dyestuff of formula: Yellow which is disclosed in GB-A-847181,
   and the dyestuff of formula: Golden yellow which is disclosed in GB-A-1171803.

Also included in the group of partially dischargeable dyestuffs are the miscellaneous dyestuffs of formulae: Red which is disclosed in GB-A-859899, and Red which is disclosed in GB-A-1027968, together with C.I. Disperse Red 72, C.I. Disperse Blue 139, C.I. Disperse Orange 55, C.I. Disperse Red 329 and C.I. Disperse Violet 40.

Any disperse dyestuff which undergoes chromophore destruction in the presence of alkali to an extent such as to make it suitable for a ground shade in discharge printing may be used in the present process, provided that it is free from -COOH, -S0₃H and -COOR- groups as defined in claim 1.

The sodium silicate which is used in the above process may be any of those grades of sodium silicate which are commercially available and is preferably a sodium silicate in which the molecular ratio of SiO₂ to Na₂0 is from 1.65:1.0 to 4.0:1.0. The potassium silicate which is used preferably has a molecular ratio of Si0₂ to K₂0 of from 2.0:1 to 4.0:1.

The amount of sodium or potassium silicate which is used in the printing paste (I) must provide sufficient alkali to discharge the disperse dyestuff in the padding liquor or printing paste (ii), and may be from 50 to 300 parts by weight per 1000 parts by weight of printing paste.

It is found that a sodium or potassium silicate having a high molecular ratio of SiO₂ to Na₂0 or K₂0 can be replaced in the printing paste by a smaller quantity of sodium or potassium silicate having a lower molecular ratio of Si0₂ to Na₂0 or K₂0, without affecting the result.

The printing paste containing the sodium or potassium silicate may also contain a humectant such as ethylene glycol urea or, preferably, glycerol, a dye solvent such as polyethylene glycol, for example, a polyethylene glycol having a molecular weight in the region of 300, and a thickening agent. The latter must be stable to the other ingredients of the paste, and examples of suitable thickeners are starch derivatives such as starch ethers, carob-seed gum ethers, modified carboxymethylcelluloses and combinations of these, optionally in admixture with water-in-oil or oil-in-water emulsion.

The padding liquor or print paste used to apply the alkali-dischargeable disperse dyestuff will also contain a carboxylic acid, for example, citric acid, to prevent premature interaction of the dyestuff with the alkaline sodium or potassium silicate, and may contain a thickener such as one of those thickeners already mentioned above. There may also be present any of those adjuvants which are conventionally employed in the application of disperse dyestuffs to synthetic textile materials from such media, for example carriers, fixation assistants, level dyeing assistants, dispersing agents and antifoam agents.

The heat treatment to which the textile material is subjected after the application of the print paste containing the sodium or potassium silicate and the print paste or padding liquor containing the disperse dyestuff can comprise a heat treatment for a short period at temperatures from 150° to 220°C. It is, however, preferred to subject the textile material to a steaming treatment, for example, saturated steam at 100°C for a few minutes followed by a dry heat treatment at 160° to 220°C or superheated steam at 150° to 200°C, or the use of saturated steam under pressure at 115° to 150°C.

The final washing stage of the process is conveniently carried out in the following sequence:-
(i) Cold water rinse.
(ii) Treatment in an aqueous alkaline bath at the pH above 8.0 and at a temperature from 50° to 85°C.
(iii) Rinse in water at 60°C.
(iv) Treatment in an aqueous bath containing 0.2% of sodium hydroxide and 0.2% of sodium hydrosulphite at 60°C.
(v) Treatment in an aqueous solution containing 0.2% of a non-ionic detergent at 60°C.
(vi) Cold water rinse, after which the. textile material is dried.

The synthetic textile material used in the process of the invention can be in the form of nonwoven fabric, felt, woven or knitted goods, or carpets. As examples of synthetic textile materials there may be mentioned secondary cellulose acetate and cellulose triacetate, polypropylene, acrylic, polyamide, and preferably aromatic polyester textile material. If desired, the synthetic textile material can be in the form of a blend or union with a cellulose textile material, for example a polyethylene= terephthalate/cotton blend or union. In the case of such blends or unions the alkali-dischargeable disperse dyestuff can be used together with a reactive dye whose reactive groups, such as sulphato- ethylsulphone groups, form a dye-fibre bond with the hydroxyl groups of the cellulose textile material which is hydrolysed under the alkaline conditions in those areas where the alkaline print paste is applied, or a reactive dyestuff containing one or more phosphonic acid groups which does not fix on cellulose in the presence of alkali.

The disperse. dyestuff or dyestuffs which are optionally used in the alkaline printing paste containing sodium or potassium silicate can be any of the disperse dyestuffs free from -S0₃H, --COOH and ―COOR groups (as defined in claim 1) and not adversely affected by alkali which are conventionally employed in colouring synthetic textile materials. Examples of such dyestuffs are given in, for example, the Third Edition of the Colour Index which was published in 1971.

The invention is illustrated by the following Examples in which parts and percentages are by weight.

### Example 1

A resist print paste comprising:

is printed on to a woven polyethylene terephthalate textile material, and without drying the textile material is then coated over all, including that part which has already been printed with the above resist paste, with the following print paste comprising:
Dyestuff of the formula:

The textile material is then dried on drying cylinders for 2 minutes at approximately 95°C, high temperature steamed at 170°C, for 8 minutes, washed off using the six-stage washing sequence described above and finally dried.

The resulting blue on white pattern has excellent definition.

If the above procedure is repeated using sodium carbonate, sodium hydroxide or potassium carbonate in place of sodium silicate the resulting prints have poor definition, bleeding-out of the alkali producing an unacceptable dull white halo round the edge of the blue areas of the print.

If the sodium silicate used in the above example is replaced by the same amount of a sodium silicate in which the molecular ratio of Si0₂ to Na₂0 is 1.65:1.0 a similar result is obtained; the amount of this latter sodium silicate can also be reduced to 100 parts without adverse effect on the sharpness of the resulting print.

Instead of the white resist print paste used in the first stage of this Example there is used a similar print paste containing, in addition to the ingredients specified above, one of the following disperse dyestuffs which are not sensitive to alkali: C.I. Disperse Yellow 63, C.I. Disperse Orange 96, C.I. Disperse Red 91, C.I. Disperse Red 210, C.I. Disperse Red 303, C.I. Disperse Blue 185, C.I. Disperse Blue 83, C.I. Disperse Red 11, C.I. Disperse Blue 95 and C.I. Disperse Violet 26. In each case there is obtained a final print having the appropriately coloured pattern on a blue ground shade. The prints have excellent definition with no haloing effect, no bleeding of the illuminant dyestuff and with bright illuminant shades.

The words "Calgon", "Manutex" and "Solvitose" are Registered Trade Marks.

### Example 2

The procedure is repeated except that the dyestuff used in the second print paste is replaced by an equal weight of any one of the other dyestuffs hereinbefore specifically identified.

In each case there is obtained a pattern having excellent definition between the discharged and undischarged areas of the print.

## Claims

1. A process for producing resist or discharge printing effects on a synthetic textile material which comprises applying to the textile material, in either order (i) an alkaline printing paste which may contain one or more disperse dyestuffs free from sulphonic acid, carboxylic acid and carboxylic acid ester groups, the said dyestuffs being unaffected by alkali at the concentration present, and (ii) a printing paste or padding liquor containing at least one alkali dischargeable disperse dyestuff free from sulphonic acid and carboxylic acid groups, and free from carboxylic acid ester groups which if hydrolysed would leave free carboxylic acid groups attached to the dyestuff molecule, thereafter heating or steaming the material and thereafter washing the material characterised by the presence of sodium or potassium silicate in (i), a carboxylic acid in (ii) and without drying between the application of (i) and (ii).

2. A process as claimed in claim 1 wherein the alkali-dischargeable disperse dyestuff is selected from one of the following classes:
A. Dyestuffs which contain one or more lactone rings which open in the presence of alkali with formation of the water-soluble alkali metal salt of the corresponding hydroxy carboxylic acid.
B. Methine dyestuffs containing at least one group.
C. Azo dyestuffs derived from anilines having at least two electron-withdrawing groups ortho and/or para to the amino group as diazo components and para-coupling amine coupling components.
D. Dyestuffs containing groups which are capable of water-soluble salt formation in the presence of strong alkali.
E. Azo dyestuffs derived from 2-aminothiophenes as diazo components and para-coupling amines as coupling components, the thiophene nucleus being substituted by at least two electron-withdrawing groups.
F. Azo dyestuffs derived from 2-amino-5-nitrothiazole as diazo component and a para-coupling amine as coupling component.
G. Miscellaneous dyestuffs selected from the dyestuff having the formula: the dyestuff having the formula: and C.I. Disperse Violet 88, C.I. Disperse Yellow 180, C.I. Disperse Violet 48, C.I. Disperse Blue 92, C.I. Disperse Yellow 93, C.I. Disperse Yellow 201, C.I. Disperse Yellow 88, C.I. Disperse Yellow 210, C.I. Disperse Red 203, C.I. Disperse Yellow 202, C.I. Disperse Red 72, C.I. Disperse Blue 139, C.I. Disperse Orange 55, C.I. Disperse Red 329 and C.I. Disperse Violet 40.

3. A process as claimed in claim 1 or claim 2 wherein the sodium silicate has a molecular ratio of SiO, to Na₂0 from 1.65:1.0 to 4.0:1.0, and the potassium silicate has a molecular ratio of Si0₂ to K₂O from 2.0:1.0 to 4.0:1.0.

4. A process as claimed in any one of claims 1 to 3 wherein the printing paste containing the sodium or potassium silicate also contains a humectant and a thickening agent.

5. A process as claimed in any one of claims 1 to 4 wherein the printing paste containing the sodium or potassium silicate also contains a dye solvent.

## Revendications

1. Procédé pour produire des effets d'impression par réserve ou rongeage sur une matière textile synthétique qui comprend l'application, sur la matière textile, dans un ordre quelconque, (i) d'une pâte d'impression alcaline qui peut contenir un ou plusieurs colorants dispersés exempts de radicaux acide sulfonique, acide carboxylique et ester d'acide carboxylique, ces colorants n'étant pas affectés par l'alcali à la concentration en présence, et (ii) d'une pâte d'impression ou liqueur de foulardage contenant au moins un colorant dispersé susceptible de rongeage par les alcalis qui est exempt de radicaux acide sulfonique et acide carboxylique et exempt de radicaux ester d'acide carboxylique qui, s'ils étaient hydrolysés, laisseraient subsister des radicaux acide carboxylique libres fixés sur la molécule de colorant, puis le chauffage ou le vaporisage de la matière et ensuite le lavage de la matière, caractérisé par la présence de silicate de sodium ou de potassium dans (i), d'un acide carboxylique dans (ii), et sans séchage entre l'application de (i) et (ii).

2. Procédé suivant la revendication 1, dans lequel le colorant dispersé susceptible de rongeage par les alcalis est choisi dans l'une des classes suivante:
A. Colorants qui contiennent un ou plusieurs cycles lactoniques qui s'ouvrent en présence d'un alcali avec formation des sels de métaux alcalins hydrosolubles de l'acide hydroxycarboxylique correspondant.
B. Colorants méthiniques contenant au moins un radical =C(CN)₂.
C. Colorants azoïques issus d'anilines portant au moins deux radicaux électronégatifs en positions ortho et/ou para par rapport au radical amino comme constituants diazoïques et d'amines copulant en para comme constituants de copulation.
D. Colorants contenant des radicaux qui sont capables de former des sels hydrosolubles en présence d'un alcali fort.
E. Colorants issus de 2-aminothiophènes comme constituants diazoïques et d'amines copulant en para comme constituants de copulation, le noyau thiophène étant substitué par au moins deux radicaux électronégatifs.
F. Colorants azoïques issus du 2-amino-5-nitro-thiazole comme constituant diazoïque et d'une amine copulant en para comme constituant de copulation.
G. Colorants divers choisis parmi le colorant de formule: le colorant de formule: le violet dispersé C.I. 88, le jaune dispersé C.I. 180, le violet dispersé C.I. 48, le bleu dispersé C.I. 92, le jaune dispersé C.I. 93, le jaune dispersé C.I. 201, le jaune dispersé C.I. 88, le jaune dispersé C.I. 210, le rouge dispersé C.I. 203, le jaune dispersé C.I. 202, le rouge dispersé C.I. 72, le bleu dispersé C.I. 139, l'orangé dispersé C.I. 55, le rouge dispersé C.I. 329 et le violet dispersé C.I. 40.

3. Procédé suivant la revendication 1 ou 2, dans lequel le silicate de sodium présente un rapport moléculaire du Si0₂ au Na₂0 de 1,65:1,0 à 4,0:1,0, et le silicate de potassium présente un rapport moléculaire du Si0₂ au K₂O de 2,0:1,0 à 4,0:1,0.

4. Procédé suivant l'une quelconque des revendications 1 à 3, dans lequel la pâte d'impression contenant le silicate de sodium ou de potassium contient aussi un humectant et un épaississant.

5. Procédé suivant l'une quelconque des revendications 1 à 4, dans lequel la pâte d'impression contenant le silicate de sodium ou de potassium contient aussi un solvant du colorant.

## Patentansprüche

1. Verfahren zur Erzeugung von Reserve- oder Ätzdruckeffekten auf einem synthetischen Textilmaterial, bei welchem auf das Textilmaterial in beliebiger Reihenfolge (1) eine alkalische Druckfarbe, die mindestens einen Dispersionsfarbstoff enthalten kann, der frei von Sulfonsäure-, Carbonsäure- und Carbonsäure-estergruppen ist und durch Alkali in der vorliegenden Konzentration nicht angegriffen wird, und (2) eine Druckfarbe oder Klotzflüssigkeit, die mindestens einen Dispersionsfarbstoff enthält, der durch Alkali ätzbar und frei von Sulfonsäure-und Carbonsäuregruppen und auch frei von Carbonsäureestergruppen ist, die beim Hydrolisieren freie, an das Farbstoffmolekülgeknüpfte Carbonsäuregruppen zurücklassen, aufgebracht wird, worauf das Material erhitzt oder gedämpft und schließlich gewaschen wird, gekennzeichnet durch die Anwesenheit von Natrium-oder Kaliumsilicat in (1) und einer Carbonsäure in (2) und das Fehlen einer Trocknung zwischen dem Aufbringen von (1) und (2).

2. Verfahren nach Anspruch 1, bei welchem der durch Alkali ätzbare Dispersionsfarbstoff aus einer der folgenden Klassen ausgewählt wird:
a) Farbstoffe, die mindestens einen Lactonring enthalten, der sich in Gegenwart von Alkali unter Bildung des wasserlöslichen Alkalimetallsalzes der entsprechenden Hydroxycarbonsäure öffnet,
b) Methinfarbstoffe, die mindestens eine Gruppe der Formel enthalten,
c) Azofarbstoffe, die sich von Anilinen mit mindestens zwei elektronenabziehenden Gruppen in ortho- und/oder para-Stellung zur Aminogruppe als Diazokomponenten und in para-Stellung kuppelnden Aminen als Kupplungskomponenten ableiten,
d) Farbstoffe, die Gruppen enthalten, welche in Gegenwart von starkem Alkali zur Bildung von wasserlöslichen Salzen fähig sind,
e) Azofarbstoffe, die sich von 2-Aminothiophenen als Diazokomponenten und in para-Stellung kuppelnden Aminen als Kupplungskomponenten ableiten, wobei der Thiophenkern durch mindestenszwei elektronenabziehende Gruppen substituiert ist.
f) Azofarbstoffe, die sich von 2-Amino-5-nitrothiazol als Diazokomponente une einem in para-Stellung kuppelnden Amin als Kupplungskomponente ableiten, und
g) verschiedenen Farbstoffen, die ausgewählt sind aus dem Farbstoff der Formel dem Farbstoff der Formel und C.I. Disperse Violet 88, C.I. Disperse Yellow 180, C.I. Disperse Violet 48, C.I. Disperse Blue 92, C.I. Disperse Yellow 93, C.I. Disperse Yellow 201, C.I. Disperse Yellow 88, C.I. Disperse Yellow 210, C.I. Disperse Red 203, C.I. Disperse Yellow 202, C.I. Disperse Red 72, C.I. Disperse Blue 139, C.I. Disperse Orange 55, C.I. Disperse Red 329 und C.I. Disperse Violet 40.

3. Verfahren nach Anspruch 1 oder 2, bei welchem das Natrium-silicat ein Molekularverhältnis von Si0₂ zu Na₂0 von 1,65:1,0 bis 4,0:1,0 und das Kaliumsilicat ein Molekularverhältnis von Si0₂ zu K₂0 von 2,0:1,0 bis 4,0:1,0 aufweist.

4. Verfahren nach einem der Ansprüche 1 bis 3, bei welchen die Druckfarbe, die das Natrium-oder Kaliumsilicat enthält, auch ein Feuchthaltemittel und ein Eindickungsmittel enthält.

5. Verfahren nach einem der Ansprüche 1 bis 4, bei welchen die Druckfarbe, die das Natrium-oder Kaliumsilicat enthält, auch ein Farbstofflösungsmittel enthält.
